

Nov. 17, 1925.

1,561,482

N. E. PHILLIPS  
CARBURIZING PROCESS  
Filed Aug. 27, 1923

*Fig. 1*



*Fig. 2*



By Inventor  
Nora E. Phillips,  
by Burton Burton Inc. Attoys.

## UNITED STATES PATENT OFFICE.

NORA E. PHILLIPS, OF CHICAGO, ILLINOIS.

## CARBURIZING PROCESS.

Application filed August 27, 1923. Serial No. 659,501.

*To all whom it may concern:*

Be it known that I, NORA E. PHILLIPS, a citizen of the United States, having residence at Chicago, in the county of Cook and the State of Illinois, have invented certain new and useful Improvements in Carburizing Processes, of which the following is a specification, reference being had to the accompanying drawings, forming a part

thereof.

The purpose of this invention is to provide an improved method and process of carburizing ferriferous metal, as cast iron, malleable or wrought iron. It consists in the employment of the materials indicated and the steps of the operation as hereinafter fully described, all as indicated in the claims.

The drawing shows an apparatus suitable for carburizing in accordance with the invention, Figure 1 being a vertical longitudinal section, and Figure 2 a vertical transverse section of a muffle furnace charged with a body of iron to be carburized and with the carburizing material disposed in relation thereto for effecting the carburizing according to the process of the invention.

In the practice of the invention consisting of this process, the metal to be treated, indicated at A in the drawings, is packed in charred leather, indicated at B, this packing having a thickness of from two to three inches on all sides and being surrounded with an outer layer of bone-meal or other pulverulent calcium bearing substance indicated at C, the entire package being encased in a metal box or muffle, D, which is exposed to heat in a suitable furnace or jacket, as indicated at E, and maintained at white heat of the metal, A, for a period of time which may vary from four to ten hours according to the thickness of the metal or depth of penetration for carburizing which is desired. For completely carburizing preparatory to hardening a cast iron bar one inch in thickness, the above mentioned temperature conditions should be maintained for approximately six hours.

The metal is then removed from the packing and as quickly as possible is immersed in a saturated solution of salt water for about 15 minutes, causing the formation of a loose scale; it is then removed from the salt water bath and immersed in a sulphuric acid bath to remove the scale.

Gray cast iron, treated by the above proc-

ess, is thereby rendered suitable in respect to carburization, hardness, and capacity for tempering, for ordinary tool purposes; and the texture is rendered such that a milling 60 cut presents the appearance of a milled surface of a good quality of tool steel.

Malleable iron castings and wrought iron, treated by this process become, for all purposes requiring hardness, toughness, and 65 susceptibility to tempering, equal to the best grades of carbon steel.

In detail, the process is performed as follows: In the metal box or muffle, D, which should be from three to five inches larger in 70 each dimension than the piece or group of pieces of metal to be treated, there is first deposited and tamped in fairly hard, a layer of bone-meal, one inch deep. Upon this bed of bone-meal, there is set a temporary re- 75 tainer, F, which comprises merely encompassing walls without top or bottom, dimensioned both horizontally and vertically from four to six inches larger than the piece of metal or group of metal pieces to be treated. 80 In this retainer there is deposited and tamped down, a layer of charred leather from two to three inches deep, and upon this bed of charred leather, the metal to be treated is laid and covered with and enclosed in charred leather, tamped down fairly hard. The space around the retainer is then filled 85 with bone-meal to the level of the top of the charred leather within the retainer, the bone-meal being tamped down firmly. The re- 90 tainer is now withdrawn and the muffle box is filled to the top with bone-meal, the remaining space for the same being substantially the same as to depth of the bottom layer of bone-meal. A tight cover, D<sup>1</sup>, is 95 then applied to the muffle box, and it is placed in the furnace or other means of applying heat. For this purpose I have usually provided a brick structure such as shown at E in the drawings, forming a 100 chamber several inches larger in every dimension than the muffle box, the latter being mounted in any convenient manner in this chamber and the space around same being filled with charcoal or coke or other suitable 105 fuel, which, being ignited and maintained in burning condition by suitable draft, heats the box and contents to the temperature indicated, viz., white heat of the metal, A, being treated.

It is to be understood that the particular mechanical means of the nature of a fur-

nace for heating the muffle box and contents, is a matter of convenience, the process requiring simply that the package be maintained at white heat of the metal treated for the necessary time to cause the desired depth of temperature of the carburizing element.

I claim:—

1. The process of carburizing iron, which consists in inclosing the iron within a closely consolidated packing of pulverulent carboniferous substance of substantial thickness enclosed in a similarly consolidated packing of pulverulent calcium bearing sub-

stance, and subjecting the package to a temperature for heating the enclosed package 15 and maintaining the same at white heat of the enclosed iron for from four to ten hours according to the depth of carburization desired.

2. In the process set forth in claim 1, 20 foregoing, the employment of charred leather as the carburizing material.

In testimony whereof, I have hereunto set my hand at Chicago, Illinois, this 17th day of August, 1923.

NORA E. PHILLIPS.